

Aug. 22, 1933.

O. ROTH, JR

1,923,642

CLEANER FOR ARTICLES OF METAL

Filed Aug. 23, 1932



O. Roth, Jr.  
INVENTOR

By: *Marks & Clark*  
Attn:

## UNITED STATES PATENT OFFICE

1,923,642

## CLEANER FOR ARTICLES OF METAL

Otto Roth, Jr., Bad Ems, Germany

Application August 23, 1932, Serial No. 630,072,  
and in Germany March 24, 1930

1 Claim. (Cl. 204--7)

My invention relates to a cleaner for articles of metal by which the articles are cleaned electrolytically.

Electrolytic cleaning was performed heretofore by contacting the articles with another metal in an electrolyte. This method is inconvenient as it requires metal plates which are not always readily obtained and comparatively expensive.

It is an object of my invention to provide a handy and cheap cleaner.

To this end, I prepare a solid substance which, dissolved, yields an electrolyte, and wrap the substance in a metal foil.

The cleaning of metal articles, such as knives, forks and spoons, which are made of, or plated with, some precious metal, usually silver, is sometimes difficult. Mechanical cleaning is objectionable because it wears the articles. If they are plated, as is the rule at present, mechanical cleaning gradually removes the plating layer and the base metal below is exposed. Articles in this condition, and particularly knives, forks and spoons, are unfit for use.

The method referred to above was performed in an alkaline electrolyte in which a plate of base metal was contacted with the articles for cleaning them. On account of the difficulties with the metal plates, and also because the concentration of the electrolyte was not properly selected, the method failed.

The drawbacks of the old method are overcome according to my invention. The means required for the cleaning, i. e. the electrolyte substance and the metal foil, are a single and handy unit.

The size of the block of electrolyte substance is so determined that it yields the required quan-

tity of electrolyte if dissolved in a given quantity of water. A suitable substance is calcined soda. It is weighed as required for the quantity of water in which it is dissolved, or shaped into lozenges or the like. The weighted quantity of substance, or the block or lozenge, is wrapped in a foil of metal, usually aluminium, which protects the substance from atmospheric influences.

In this manner a handy and durable cleaner is provided.

In the accompanying drawing, a cleaner embodying my invention is illustrated by way of example.

In the drawing, 1 is the wrapper of metal foil, and 2 is the electrolyte substance, here shown as a block or lozenge. Obviously, it might also be in the condition of powder.

For using the cleaner, the foil 1 is removed from the substance 2, the substance is dissolved in the prescribed quantity of water, the solution slightly heated if desired, the foil 1 placed in the solution, and the article to be cleaned, for instance, a silver or plated spoon, is brought into contact with the foil. The dirt is soon removed in this manner and the articles are perfectly clean after having been rinsed with water.

I claim:

A method which comprises wrapping a solid body in an electro-negative metal foil, said solid body being capable of forming an electrolyte, and subsequently dissolving said solid in water to form a bath and using said foil as a source of electronegative metal in the bath for the cleaning of metal surfaces.

OTTO ROTH, JR.